

April 17, 1928.

C. J. COBERLY

1,666,166

METHOD OF CUTTING SLOTS IN METAL

Filed Dec. 2, 1925

Fig. 1.



Fig. 2.



INVENTOR:  
CLARENCE J. COBERLY,

By  
Ford A. Karr  
ATTORNEY.

## UNITED STATES PATENT OFFICE.

CLARENCE J. COBERLY, OF LOS ANGELES, CALIFORNIA, ASSIGNOR TO KOBE, INC., OF LOS ANGELES, CALIFORNIA, A CORPORATION OF CALIFORNIA.

## METHOD OF CUTTING SLOTS IN METAL.

Application filed December 2, 1925. Serial No. 72,890.

My invention relates to the art of cutting slots in metal by use of a cutting torch, and particularly to a method and apparatus whereby slots may be expeditiously and accurately cut in metal.

In an application entitled Pipe slotting machine, filed October 1, 1923, Serial No. 665,917, I have described a machine and a method whereby slots are cut in a metal by 10 use of a cutting torch. Briefly, the method consists in drilling a starting hole in the metal (which in the mentioned case was a steel pipe to be made into a well strainer) for providing a start for a slot, and cutting 15 a slot in the metal by use of a cutting torch, this slot being started at said starting hole.

I have discovered that by preheating the metal the slot may be quickly and accurately cut, since the cutting torch operates more 20 effectively on metal at a high temperature.

It is, therefore, an object of this invention to provide a method of cutting a slot in metal in which the metal is preliminarily heated and the slot is cut while the metal 25 is hot.

In my method I prefer to heat the metal after the starting hole has been drilled so that the drill may operate on cold metal, since drilling in hot metal would take the 30 temper out of the drill.

It is, therefore, another object of my invention to provide a method for forming a slot in a metal which consists in drilling a starting hole, then preliminarily heating the 35 metal and finally cutting the slot.

It is another object of this invention to provide an apparatus for forming slots in a metal, having a means for heating the metal before the cutting of the slot.

It is a further object of this invention to provide an apparatus of the character mentioned having a heater in the form of an induction heater.

I have further found that in cutting slots in steel pipe, the hardness of the surface of the slot depends on the rate of cooling after the cutting flame has passed and on the analysis of the steel, particularly the carbon content. In slotting the low carbon steels used in welded pipe, the cooling due to the flow of heat to the metal back of the heated zone, has a very beneficial effect on the physical properties of the metal, greatly in-

creasing the hardness and strength. In some cases it is desirable to increase the rate of cooling by quenching with an air blast or other means, as disclosed in my application Serial No. 665,917. In slotting steel of higher carbon content (.40% to .60% carbon) as are sometimes used in making seamless steel pipe, the above means of quenching causes too great an increase in hardness and a reduction of ductility, in some cases even causing microscopic cracks on the surface of the slot which are detrimental in that they form favorable places for a fracture to start. In other words, the hardness is increased to a point where the metal is brittle, which is undesirable in slotted pipe subject to severe strain and abrasion.

I have found that this hardness can be controlled and that the metal around the slot can be made stronger and harder than the original metal without loss of ductility by proper control of the initial temperature of the steel. This works in two ways to accomplish the desired result. First, the metal being initially at an elevated temperature is equivalent to drawing the temper after quenching. Second, and more important, the rate of conduction of heat from the metal in the zone raised to a very high temperature by the cutting action is greatly reduced by increasing the initial temperature of the steel. Hence, raising the initial temperature of the steel 500° F. is much more effective than raising it to this temperature as a second operation after cutting.

In comparing this process with the usual methods of heat-treating steel, it should be remembered that it differs fundamentally in that the metal is heated rapidly above the critical and then cooled rapidly. The high temperature is not sustained as is customary in the usual heat-treatment. The structure and physical properties of the metal depend upon both the rate of heating and rate of cooling, and both of these things are controlled by means of the initial temperature of the steel.

It is accordingly an object of this invention to provide a method of heat-treating steel as previously explained and particularly at the time slots are formed therein. By means of this process it is possible to accurately control the conditions so as to ob-

tain the maximum hardness and toughness for each grade of steel with the result that the resistance to sand abrasion and the strength of the casing are greatly increased.

5 Other objects and advantages of my invention will be made evident hereinafter.

Referring to the drawings in which I illustrate an apparatus whereby my invention may be carried out,

10 Fig. 1 is a cross section through an apparatus of my invention.

Fig. 2 is a section taken on the line 2—2 of Fig. 1.

15 The form of apparatus shown in the drawings is adapted to cut slots in a pipe indicated at 11. A frame 12 surrounds the pipe 11. This frame 12 consists of annular plates 13 and 14 which are secured together by a cylindrical member 17 having 20 flanges 18 which are secured to adjacent faces of the plates 13 and 14 by suitable cap screws 19.

25 Secured to the outer face of the plate 14 in any suitable manner is a plurality of drill devices 20 having drills 21. The devices 20 have pulleys 22 which are operated by belts (not shown) for rotating the drills 21. The drill devices 20 are constructed so that the drills 21 may be automatically fed into the 30 wall of the pipe 11 in order to form starting holes 24 and also to be automatically withdrawn therefrom. The drill devices 20 may be of the same construction as shown in my application mentioned in the preamble of 35 this specification.

Extending inwardly from the cylindrical member 17 is an annular flange 27 to which an annular flange 28 of an induction heater 30 is secured by screws 31. This induction 40 heater 30 has coils 33, 34, and 35, which have wires 37 of a three-phase circuit connected thereto. Also connected to the coils 33, 34 and 35 are ground wires 38 which extend to a ground, as diagrammatically indicated in Fig. 1. The coils 33, 34 and 35 are annular and completely surround the pipe, as shown in Fig. 2. When the coils are energized, magnetic lines of force are set up, which lines of force set up induced 45 electric currents in the wall of the pipe 11, heating it to the desired temperature.

50 Secured to the outer face of the annular plate 13 of the frame 12 is a plurality of cutting torches 40. The cutting torches 40 have tips 41 which are positioned adjacent to the wall of the pipe 11. The cutting torches 40 are supplied with oxygen and acetylene gas through conduits 42 and 43. The tips 41 of the torches 40 are so positioned 55 as to align with the starting openings 24 produced by the drills 21 and are adapted to form slots in the pipe 11, as indicated at 45.

55 A complete operation of my invention is substantially as follows:

The induction heater 30 is set into operation by supplying electricity therethrough to the wires 37 which set up magnetic lines of force which cut the wall of the pipe 11 and induce electric currents therein which 75 raise it to the proper temperature, which is preferably such as will permit the torches to readily heat the pipe to an oxidizing temperature. The drill devices 20 are set into operation and the drills 21 are rotated and 75 fed inwardly into the wall of the pipe 11 in a manner to produce the starting holes 24. The drills 21 are withdrawn. The tips 41 of the cutting torches 40 are at this time in alignment with a series of starting holes 24. 80 The torches 40 are then lighted by automatic means. The frame 12 is supported by means (not shown) whereby it may be moved along the pipe 11 in a right hand direction. As the frame 12 moves, the cutting jets produced by the torches 40 are moved therewith and slots 45 are formed by the action of the jets of the torches. The frame 12 is moved through a sufficient distance to provide the desired length of slot. The 90 frame is then stopped and the torches 40 are shut down. The drill devices 20 are again set into operation and the sequence of operations just described is repeated.

95 As previously mentioned, by providing the heater 30 for preheating the pipe 11 it is possible to quickly cut the slots 45 and to cut them very accurately, so that they will have very smooth walls and will be of a uniform size which is highly desirable. My invention is very well suited for use in making well strainers for the oil well industry and it is very desirable to have the slots in well strainers of a uniform size. It is well known in the welding industry that in order 100 to cut metal, it is necessary to preheat it to a temperature which approaches the fusing point of the metal, so that the oxygen when supplied to the torch will be able to burn the metal away. By using the heater 30 it 110 is possible to raise the temperature of the pipe 11 to a desirable temperature so that the metal may be readily and effectively burned away.

115 Another important advantage of the invention is the hardening of the metal, which is advantageous especially when the pipe is used as a well strainer because oil generally carries small particles of abrasive which tend to wear away the walls of the slots. The induction heater very quickly raises the temperature to a determined degree which is highly desirable, and the metal will cool evenly and at a uniform rate. The heater may be regulated to heat the pipe to any desirable temperature and the hardening of the pipe may be thus controlled. After the walls of these slots are hardened, they will resist the attritional action of the abrasive particles. The heater 30 is placed be- 120 125 130

tween the drill devices 20 and the torches 40 so that the pipe 11 will be heated after the starting holes are produced so that the drill 21 will operate on cold metal and so that the 5 temper will not be taken therefrom.

I claim as my invention:

1. A method of forming a slot in a piece of metal and determining the rate of quench of the walls of said slot, said method comprising: uniformly heating an extensive area of said metal; directing a cutting jet through said metal in an interior portion of said extensive heated area to form a slot in said metal, the difference in temperature between 10 the walls of said slot and said extensive area of metal being much less than otherwise, due to said uniform heating of said extensive area; and permitting said metal to cool gradually, the temperature of said extensive 15 area determining the rate of quench of the walls of said slot.

2. A method of forming a slot in a piece of metal and determining the rate of quench of the walls of said slot, said method comprising: heating an extensive area of said metal; directing a cutting jet through said metal in an interior portion of said extensive heated area to form a slot in said metal, the difference in temperature between the walls 20 of said slot and said extensive area of metal being much less than otherwise, due to said heating of said extensive area; and permitting said metal to cool gradually, the temperature of said extensive area determining 25 the rate of quench of the walls of said slot.

3. A method of slotting pipe, said method comprising: forming starting holes in said pipe; substantially uniformly heating an extensive zone of said pipe; directing cutting jets through certain holes in said zone; moving said pipe relative to said jets whereby slots are formed in an interior portion of 30 said zone; and allowing said pipe to cool gradually, the heat applied to said zone preventing too rapid cooling of the walls of said 35 slots.

4. A method of slotting high carbon steel pipe, said method comprising: forming starting holes in said pipe; substantially uniformly heating an extensive zone of said pipe to a temperature above 400° F.; directing cutting jets through certain holes in said zone; moving said pipe relative to said jets whereby slots are formed in an interior 40 portion of said zone; and allowing said pipe to cool gradually, the heat applied to said 45

zone preventing too rapid cooling of the walls of said slots.

5. A method of slotting pipe, said method comprising: forming starting holes in said pipe; substantially uniformly heating an annular zone of said pipe; directing cutting jets through certain holes in said zone; moving said pipe relative to said jets whereby slots are formed in an interior portion of 50 said zone; and allowing said pipe to cool gradually, the heat applied to said zone preventing too rapid cooling of the walls of 55 said slots.

6. A method of slotting pipe, said method comprising: causing heat rays to converge toward a given space; forming a hole in a zone of a pipe; extending said zone into said space, for a sufficient length of time to heat said zone uniformly to a given temperature; forming a hole in a portion of said pipe which has not yet been extended into said heating space, while said zone is being heated; moving said pipe to a new hole-forming and heating position; and directing 60 a cutting jet through the hole in said zone while said pipe is being moved in order to form a slot in said zone.

7. A method of cutting a slot in metal with a wall of predetermined hardness said method comprising: preheating an extensive area of said metal to a desired temperature; directing a cutting jet through said metal in said extensive area to form a slot in said area; and permitting said metal to cool so 70 as to quench a wall of said slot, the length of time consumed by said quenching being determined by the difference between the temperature given said wall in the cutting of said slot and the temperature to which 75 said extensive area was heated.

8. A method of forming a slot in metal and controlling the hardness of a wall of said slot said method comprising: uniformly heating an extensive area of said metal; directing a cutting jet through said metal in said extensive heated area to form a slot in said metal; and quenching a wall of said slot, the difference between the temperature given said wall in the cutting of said slot 80 and the temperature to which said extensive area was uniformly heated affecting the rate 85 of quench of said wall.

In testimony whereof, I have hereunto set my hand at Los Angeles, California, this 110 25 day of November, 1925.

CLARENCE J. COBERLY.